

Jan. 24, 1950

O. R. HOELTZEL ET AL

2,495,636

INSULATING PAD

Original Filed May 22, 1944

FIG. 1



FIG. 2



Inventor's  
Orval R. Hoeltzel  
William S. Saville  
John W. Larson

By Fred Gerlach their Atty.

## UNITED STATES PATENT OFFICE

2,495,636

## INSULATING PAD

Orval R. Hoeltzel, William S. Saville, and John W. Larson, Fort Worth, Tex., assignors to Consolidated Vultee Aircraft Corporation, San Diego, Calif., a corporation of Delaware

Original application May 22, 1944, Serial No. 536,768. Divided and this application February 10, 1945, Serial No. 577,274

3 Claims. (Cl. 154—44)

1

The invention relates to insulating pads and method of making such pads.

In aircraft, it has been found desirable to insulate and sound proof the walls by pads which may be readily installed on the walls and removed therefrom when repairs are necessary.

One object of the invention is to provide an improved insulating and sound-proofing pad of the construction which is adapted for removable installation in aircraft, can be handled with facility during installation or removal, and is light in weight.

Another object of the invention is to provide an insulating and sound-proofing pad which comprises a mat of fiber and a tough protective film for one face of the pad for making this area impervious to moisture and air.

Another object of the invention is to provide a pad which includes a bat or mat of fibrous material and a protective film integralized with the fiber of the mat and which does not substantially add to the overall weight of the pad.

Other objects of the invention will appear from the detailed description.

The invention consists in the several novel features hereinafter set forth and more particularly defined by claims at the conclusion hereof.

In the drawings:

Fig. 1 is a perspective of a pad embodying the invention.

Fig. 2 is a transverse section taken on line 2—2 of Fig. 1.

The invention is exemplified in a pad which comprises a layer or mat 8 of loosely matted suitable fibrous material, such for example as fiber-glass; a flexible film or septum 9 of plastic material which is directly integralized with or bonded to the fibers in one face of the fibrous material; and a finishing face 10 of suitable fabric. The fabric facing 10 consists of a sheet which is folded around the margins of the mat as at 13, and to overlie as at 14 the outer face of the film, and secured together by a seam 11 which extends through the face covering portion and enfolded margin of the fabric and the integralized mat and film. Sockets 12 of stud and snap fasteners are secured in the corner of the pad and are adapted to be connected to matting studs (not shown) which are secured in the wall which is to be covered by pads. The pads may be formed of any suitable contour and size to form sections which completely cover the wall or a section thereof. The pad is placed with the film 9 next to the wall and is impervious to moisture and sound. The fabric forms a finished wall surface when the

2

pads are secured in multiple on the wall and adjacent to each other.

The film or septum 9 consists of a flexible and soluble plastic material such as a rubber hydrohalide such as rubber hydrochloride. The film is bonded to the fiber-glass while it has been softened to a semi-fluid condition by a suitable solvent to render it adhesive so it will bond to and embrace fibers to which it is applied when the solvent is evaporated and the film is dried and set or hardened and becomes integralized with the fibers.

The film is integralized with the matted layer of fiber-glass by softening the film with a suitable solvent such as methyl-ethyl-ketone, to render it adhesive, subjecting the softened film and matted layer to heat to accelerate the action of the solvent, and to pressure and vacuum to force the film into close contact with the fibers and then subjected to heat to dry and set the film on the fibers as set forth in our application filed May 22, 1944, Serial No. 536,768, of which the present application is a division. During this bonding the film is bonded to and integralized with the fibers of the mat. The surface of the film becomes wrinkled or wavy which results from its stretching while it is soft and during its integralization with the fibrous mat.

A sheet of the textile fabric 10 is then cut to the shape of the pad desired with a projecting marginal portion for a fold around the edges of the integralized film and fibrous material. The sheet of fabric is then placed over the bare face of fibrous material and its marginal portion 14 is folded around the edges of the combined sheet of film and layer of fibers. The portion 14 and the marginal portion of the face-portion of the fabric 10 with the integralized film and fibrous material between them are stitched together by the seam 11. The folded edge of the fabric, outwardly of the fibrous material, may also be stitched together by a seam 21. The sockets 12 for the stud fasteners, in desired number, are then secured to the corners or other portions of the mat so the pad can be initially and readily attached to the matting studs secured in the wall structure of the aircraft, and so that the pad will be held against said structure. The pads are secured on the wall in edge to edge relation to cover the wall or portion thereof which required insulation.

The invention exemplifies an insulating pad which comprises matted fibrous material, preferably fiber-glass, and a flexible film of plastic material which forms a protective covering which

is integralized with the matted fibrous material. The pad is light in weight, is an efficient sound and moisture insulation and is provided with a finishing face of insulation on the walls. The flexibility of the pads adapts it to conform to walls of different contour on which it is installed.

The invention provides an insulating and sound-proofing pad which comprises a mat of fiber and a tough protective film for one face of the pad for making this face withstand rough handling and retain a high fatigue value over a substantial cycle in installation and removal of the pad.

The invention is not to be understood as restricted to the details set forth since these may be modified within the scope of the appended claims without departing from the spirit and scope of the invention.

Having thus described the invention, what we claim as new and desire to secure by Letters Patent is:

1. A unit comprising a layer of loosely matted mass of fibrous material, a substantially impervious, preformed film of thermoplastic synthetic resin material integralized with the fibers in one face of the loosely matted material, a fabric covering the other face of said loosely matted layer and enfolded and secured around the edges of the mass and the film, the mass, film, and fabric being in the form of a sound-proof, flexible pad adapted to cover and sound-proof a section of a wall, and means for readily and demountably securing the pad on the wall.

2. A unit comprising a layer of loosely matted mass of glass fibers, a substantially impervious, preformed film of thermoplastic material integralized with the fibers in one face of the loosely matted material, a fabric covering the other face of said loosely matted mass and enfolded and secured around the edges of the mass and the film,

5 the mass, film, and fabric being in the form of a sound-proof, flexible pad adapted to cover and sound-proof a section of a wall, and means for readily and demountably securing the pad on the wall.

3. A unit comprising a layer of loosely matted mass of glass fibers, a substantially impervious, preformed film of rubber hydrohalide integralized with the fibers in one face of the loosely matted material, a fabric covering the other face of said loosely matted mass and enfolded around the edges of the mass and the film, the mass, film and fabric being formed into a sound-proof, flexible pad adapted to cover and sound-proof a section of a wall, and means for readily and demountably securing the pad on the wall.

ORVAL R. HOELTZEL.  
WILLIAM S. SAVILLE.  
JOHN W. LARSON.

#### REFERENCES CITED

The following references are of record in the file of this patent:

#### UNITED STATES PATENTS

| Number       | Name         | Date           |
|--------------|--------------|----------------|
| 1,484,056    | Birtch       | Feb. 19, 1924  |
| 2,086,433    | Prudden      | July 6, 1937   |
| 2,108,682    | Leslie       | Feb. 15, 1938  |
| 2,215,061    | Alt          | Sept. 17, 1940 |
| 2,249,275    | Hanley       | July 15, 1941  |
| 2,252,157    | Bergin       | Aug. 12, 1941  |
| 2,273,452    | Snyder       | Feb. 17, 1942  |
| 2,355,608    | Stieger      | Aug. 15, 1944  |
| 35 2,381,542 | Hyatt et al. | Aug. 7, 1945   |

#### FOREIGN PATENTS

| Number  | Country       | Date          |
|---------|---------------|---------------|
| 482,809 | Great Britain | Apr. 5, 1938  |
| 527,570 | Great Britain | Oct. 11, 1940 |